

L. T. GROUSSELLE.

MANUFACTURE OF STEEL DIRECT FROM IRON ORES.

APPLICATION FILED AUG. 4, 1917.

1,284,094.

Patented Nov. 5, 1918.



INVENTOR  
Luis Tejero Grouselle

BY *Paul Mainely, Jr.*  
ATTORNEY

# UNITED STATES PATENT OFFICE.

LUIS TEJERO GROUSELLE, OF GRENOBLE, FRANCE.

MANUFACTURE OF STEEL DIRECT FROM IRON ORES.

1,284,094.

Specification of Letters Patent. Patented Nov. 5, 1918.

Application filed August 4, 1917. Serial No. 184,479.

*To all whom it may concern:*

Be it known that I, LUIS TEJERO GROUSELLE, a subject of the King of Spain, residing at Grenoble, France, 39 Rue Lesdiguières, have invented certain new and useful Improvements in the Manufacture of Steel Direct from Iron Ores, of which the following is a specification.

My invention relates to a furnace for producing steel direct from iron ores.

The objects of my invention are:—

(1) To obtain the same reactions as in the blast furnace, but without any contact with free carbon, in order that the operation, when completed, should produce steel, and not cast iron;

(2) That the temperature should be as high as, if not higher than, that in the ordinary blast furnace;

(3) That the consumption of fuel should be less than that in the ordinary blast furnace.

In the drawing,

Figure 1 is a vertical section of the apparatus,

Fig. 2 is an elevation in a plane at a right angle to Fig. 1, half in section, and

Fig. 3 is a plan.

The apparatus comprises a sort of blast furnace provided with a hearth, the whole of more or less great dimensions according to the quantity of ore to be treated, the reducing and fusion functions being entirely separated and brought about by gases of different nature.

In a refractory masonry body *a* (Fig. 1) surrounded by ordinary masonry *a'* and entirely armored outside, is a chamber *b* into which projects a metal chamber *c* extended by a sleeve *c'* of refractory material. The chamber *c* is charged with ore through a hopper *d*, the inlet door *d'* and the outlet door *e* of which open alternately, the latter being opened by means of a lever with a balance weight *r* (Fig. 3), in order to prevent air from getting in, or gases from escaping, during the charging of the ore.

Through the pipe *v* is admitted hydrogen or hydrogenated gas (water gas, natural gas, etc.) generated separately, which circulates in the upward direction in the pipe *v* with internal radiation ribs, heated outside by the hot escaping gases of the furnace circulating in the downward direction in the

flue *x'*, and enters through *v'* the chamber *c*, in order to filter through the ore in the downward direction and escape through the annular space left between the chambers *c* and *c'*, and through the chimney *x'*.

The ore reduced in the chamber *c*, follows its path through *c'* and arrives at the shaft or stack *i*.

On arriving there, it is heated by the large amount of heat generated by the blow pipes of the twy whole *l*, *l*, *l*, etc., supplied with non-hydrogenated gases generated separately, and with air admitted through the orifice *p*; this air is heated by the waste heat owing to its circulation in the coil *s*; the air is admitted cold at *p* and escapes hot at *y* in order to pass to the collector *m* which distributes it to the twy whole *o*. As regards the non-hydrogenated gas (for fusion), it is admitted at *w*, passes to the collector *n* which also distributes it to the twy whole *o*.

The hearth *j* having received sufficient molten metal, the casting is effected through *a''*.

The gases coming from the twy whole *l*, *l*, *l*, etc., circulate in the fusion chamber *j* and pass through *k* and *i* to the chimney *x'* after having filtered through the reduced ore.

The draft of this apparatus is by compression, as between the gas producing apparatus and the furnace are arranged fans, forcing gases into the furnace.

The gas producers can thus work freely, and their cleaning and manipulation are facilitated.

It goes without saying that the production of the gases, the admission of the air and the temperature are regulated by valves of the twy whole, and by the more or less great admission of hydrogen or of reducing gas into the reducing chamber.

This being clearly understood, it will be seen that the apparatus thus arranged complies with all the conditions which are:

(1) To effect reduction by hydrogen or by a hydrogenated and oxycarbonated or hydrocarbureted gas, without having to fear the reverse reaction of the resulting water on the metal produced.

(2) To carburet the iron obtained, without converting it into cast iron, since the carbureting is brought about by oxid of carbon, and not by carbon, the reduction

taking place without contact with the latter, the reducing gases as well as the fusion gases being produced separately.

(3) To work with an enormous economy 5 of fuel, this being due to the process and to the use of the waste heat for heating the combustion air and the reducing gases.

(4) To offer the advantage of enabling 10 iron ore to be treated which contains impurities which render it useless for treatment by the usual processes, and any fuel to be used.

(5) To arrange a fusion and a purification chamber which offers all the necessary 15 conditions for insuring fusion and purification of the steel obtained.

(6) To work by suction and compression, which facilitates the manipulation of the furnace and of the gas producers, the whole 20 "being translated" into a guarantee of uninterrupted working.

What I claim as my invention and desire 25 to secure by Letters Patent is:—

1. In a furnace for producing steel direct from iron ores, a reducing chamber, means for introducing reducing gas therein, a melting chamber, independent means for introducing heating gases into said melting

chamber, and an exit passage way for the waste gases independently connected with 30 the reducing and melting chambers.

2. In a furnace for producing steel direct from iron ores, an upstanding stack, a reducing chamber extending longitudinally within the stack and spaced laterally therefrom 35 for providing a gas outlet passage, means for introducing iron ore into the upper end of the reducing chamber, means for introducing a reducing gas into the upper end of the reducing chamber, a tubular member 40 arranged beneath and spaced from the lower end of the reducing chamber so that said lower end has communication with said gas outlet passage, said tubular member being spaced laterally from said stack to provide 45 a second gas passage, a melting chamber arranged beneath the tubular member and discharging its gases into the second gas passage, and separate means for supplying heated gases to the melting chamber. 50

In testimony whereof I affix my signature in presence of two witnesses.

LUIS TEJERO GROUSELLE.

Witnesses:

GEORGE CONSTANT,  
ALFRED MIRALL.